

## UNITED STATES PATENT OFFICE

2,234,905

## DYEING OF CELLULOSETIC TEXTILE MATERIALS

Ernest Edward Tallis, Coventry, England, assignor to Courtaulds, Limited, London, England, a British company

No Drawing. Application November 19, 1938, Serial No. 241,460. In Great Britain November 30, 1937

4 Claims. (Cl. 8—100)

This invention relates to the dyeing of cellulosic textile materials.

It is well known that it is not ordinarily possible to dye cellulosic materials such as cotton, 5 rayon, linen or the like with acid dyestuffs such as are commonly used for the dyeing of wool and the like animal fibres.

It is also known, however, that such cellulosic fibres can be dyed by acid dyestuffs if the fibres 10 have been pretreated with various materials. For example it has been proposed to dye such cellulosic fibres after treatment with nitrogenous materials, such as amines and ammonium bases.

Treatment with solutions containing urea or 15 thiourea mixed with or precondensed with aldehyde followed by heating to obtain condensation products on the fibres has also been proposed for this purpose. It has also been stated that the methylol compounds of urea or thiourea do not 20 possess sufficient chemical affinity for acid dyes to be useful technically for dyeing purposes. In view of this a proposal has been made to use the initial condensation products of formaldehyde with dicyandiamide, guanidine or heat-treated 25 urea, which while not detrimental to the good textile properties of the fibre lend it a pronounced affinity for acid dyestuffs and in some cases for basic dyestuffs.

In British Patent No. 319,822 a process of manufacturing new compounds by the interaction of 30 cyanamide with formaldehyde is described and it is stated that the properties of the product obtained by condensing under acid conditions are different from those of the product obtained by 35 condensing under alkaline conditions.

According to the present invention the process 40 for improving the dyeing properties of cellulosic textile materials, comprises incorporating in the said materials a product obtained by causing cyanamide and formaldehyde to react under acid or neutral conditions.

One method of carrying out the said process, 45 comprises impregnating the said cellulosic textile materials with a solution, obtained by mixing in the cold solutions of cyanamide and formaldehyde, which solution is maintained slightly acid. The best results are obtained when the pH value of the solution lies between 5.0 and 6.5. After impregnation the material is dried and 50 heated to ensure reaction between the cyanamide and formaldehyde. The cyanamide and formaldehyde may be partially or wholly precondensed by heating the mixed solution at raised temperatures, for example 80° to 100° centri- 55 grade, under slightly acid conditions, preferably

at a pH value of 5.0. The material after impregnation with the solution thus obtained is dried and heated to complete the reaction between the cyanamide and formaldehyde in the material.

Alternatively, the process according to the 6 present invention, may be carried out by incorporating in the cellulosic solution, for example, viscose, which is to be used for forming cellulosic threads, the product which is precipitated on prolonged heating above 60° centigrade of a solution of the initially slightly acid solution obtained by mixing solutions of cyanamide and formaldehyde.

An intensifier or any other useful compound, 15 for example ammonium thiocyanate, which greatly increases the affinity of the textile material for certain direct dyestuffs, may be added to the solutions used for the treatment of such materials. If these intensifiers or other compounds are of a basic nature, for example, triethylamine, 20 then it is necessary to neutralise them before they are incorporated in the treating solution.

The cellulosic materials obtained according to 25 the present invention have an increased affinity for many classes of dyestuffs which may be applied to such materials, including direct cotton, sulphur, vat, azoic, basic and acid dyestuffs, and also those dyestuffs specially evolved for the dyeing of cellulose acetate or the like cellulose derivatives. Moreover, the fastness to washing 30 processes of the resulting dyed material is greatly improved.

The following examples illustrate methods of carrying the present invention into effect, although the invention is not restricted to these 35 examples.

*Example 1*

12 parts of crude calcium cyanamide are extracted with 36 parts of water at from 35° to 45° centigrade for 30 minutes and subsequently filtered and neutralised with strong sulphuric acid. The calcium sulphate is filtered off. To the filtrate are added 15 parts of commercial formaldehyde solution (containing 40 per cent of formaldehyde), 1 part of ammonium thiocyanate and 15 parts of water. Viscose staple fibre is steeped in this solution, squeezed out and centrifuged to twice its original weight. It is then dried by known processes and finally heated for twenty minutes at 140° centigrade. It is then dyed at 50 the boil for one hour with 1 per cent of azo-geranine 2 G. S. and 2 per cent of sulphuric acid. A rich scarlet shade is imparted to the fibre comparable with that developed by the same dyestuff on wool.

**Example 2**

5 A solution, containing 4 per cent of cyanamide and 3 per cent of formaldehyde, at a pH value of 5.0, is heated at 80° centigrade until a voluminous white precipitate is formed. The precipitate is filtered off, washed and dried. It is then dispersed in acetone and added to a cellulose acetate spinning solution. The cellulose acetate 10 yarn obtained from this solution is then dyed at 80° centigrade for one hour with 2 per cent azo-geranine 2 G. S., and 2 per cent of formic acid. It can also be dyed under the same conditions with erio fast cyanine S concentrated.

15

**Example 3**

20 Viscose yarn impregnated for 15 minutes at room temperature with a solution containing 4 per cent of cyanamide, 3 per cent of formalin (40 per cent formaldehyde) and 2 per cent of ammonium thiocyanate at a pH value of 6.0. The 25 impregnated yarn is then hydro-extracted, dried and heated at 150° centigrade for 5 minutes. It is then dyed a full shade with 3 per cent coomassie red P. G. S. (Imperial Chemical Industries) and exhausts the dye bath. The yarn obtained is also dyed a much fuller shade with indigosol blue I. B. C. than yarn which has not been so treated.

30

**Example 4**

35 5 parts of a 40 per cent solution of cyanamide are added to 6 parts of 40 per cent formaldehyde solution and the resulting solution is heated at 95° centigrade for 3 minutes. After rapidly cooling to room temperature the solution is diluted with 60 parts of water and the solution so obtained used to impregnate staple fibre. The 40 impregnated staple fibre is hydro-extracted and dried at 70° centigrade the temperature then be-

ing raised to 100° centigrade for one hour. The 45 treated fibre is dyed at the boil for 1/4 of an hour in a dyebath containing 2 per cent of azo-geranine 2 G. S. and 2 per cent of formic acid on the weight of the fibre using a liquor to yarn ratio of 5 40 to 1. The dyebath is exhausted and a full shade developed on the fibre.

What I claim is:

1. A process for improving the dyeing properties of cellulosic textile materials which comprises 10 incorporating in the said materials a product obtained by causing cyanamide and formaldehyde to react in a solution the pH value of which initially lies between 5.0 and 6.5.

2. A process as claimed in claim 1, wherein the 15 materials are impregnated with the solution obtained by the admixture in the cold of solutions of cyanamide and formaldehyde, which solution is maintained slightly acid at a pH value between 5.0 and 6.5, the said materials after impregnation 20 being dried and heated to cause reaction between the cyanamide and formaldehyde.

3. A process as claimed in claim 1, wherein the 25 materials are impregnated with the solution obtained by heating a solution containing cyanamide and formaldehyde while maintaining the pH value of the solution between 5.0 and 6.5 to give partial or complete precondensation, and are thereafter dried and heated to complete the reaction between the cyanamide and formaldehyde. 30

4. A process as claimed in claim 1, wherein the product which is precipitated after the prolonged heating above 60° centigrade of a solution of cyanamide and formaldehyde the pH value of which is initially between 5.0 and 6.5, is incorporated 35 in the cellulosic solution from which cellulosic textile threads are produced.

ERNEST EDWARD TALLIS.